

# UNITED STATES PATENT OFFICE.

CHARLES MORRIS JOHNSON, OF AVALON, PENNSYLVANIA.

## VAULT-PLATE.

1,342,913.

Specification of Letters Patent.

Patented June 8, 1920.

No Drawing.

Application filed August 7, 1919. Serial No. 315,960.

*To all whom it may concern:*

Be it known that I, CHARLES M. JOHNSON, residing at Avalon, in the county of Allegheny and State of Pennsylvania, a 5 citizen of the United States, have invented or discovered certain new and useful Improvements in Vault-Plates, of which improvements the following is a specification.

My invention relates to improvements in 10 vault-plates, that is to say plates out of which the walls of a safe, a safe-deposit vault or like structure may wholly or in part be built. The object in view is flame resistance. In vault building steel of great 15 hardness has heretofore been used, to resist the cutting tools employed by burglars; but such very hard steel is not sufficiently resistant to a blow-pipe flame, and in consequence such safes and the like which are strong to 20 resist cutting tools may still be penetrated with relative ease, and the blow-pipe flame has become the burglar's most effective tool. Under such conditions walls of safes and the like are now being built of compound 25 plates or layers, some of these layers being hard to resist cutting tools, and others of softer material, more resistant to cutting by flame.

I have found through long continued 30 study and experiment a steel mix, a steel alloy, which is in highest degree resistant to flame penetration, and my invention consists in a vault plate formed of such steel.

The steel alloy which I have worked out 35 belongs in the class termed chrome steel: that is to say, it is steel alloyed with chromium. Chrome steel is not new with me; nor is it new with me to use chrome steel for the walls of safes; the flame-resisting 40 property of chrome steel as a class is known—though the reason why chrome steel is flame-resisting has not, so far as I am aware, been known heretofore. I have discovered the reason to be this: Chromium 45 oxid, which under the blow-pipe flame soon covers in a layer of increasing thickness the surface attacked, is a highly refractory substance; its melting point is given as 3614° F. This layer increasingly protects the under- 50 lying metal from melting and burning through under the flame.

I do not claim to have discovered that 55 chrome steel may be used for vault plates. I have discovered that a nickel-chrome steel—a steel alloyed not with chromium only but with nickel too,—has a flame-re-

sisting capacity exceeding the simple chrome steel alloy, and furthermore, is workable—capable of being forged and sheared, drilled, and machined, etc.—with an ease 60 not enjoyed in the case of the simple alloy. Indeed, an obstacle to making plates of simple chrome steel has been the impossibility of fabricating, if the chromium content be great. For attaining the object now 65 in view, I find that, within the range of my experiments, the greater the chromium content the greater the capacity to resist flame penetration. I further find that by adding nickel to the alloy, not only do I remove 70 the obstacle mentioned,—or, rather, push it farther out of the path,—but that, instead of impairing the capacity to resist flame (a result which might have been expected), I actually improve that capacity. So I obtain 75 a new result, a steel of great flame-resisting quality which is easily workable, a vault plate which reveals a flame-resisting capacity unapproached by anything heretofore devised.

The characteristics of my vault plate material are these: First of all, it is a steel 80 alloy. That is to say, steel is the dominant element. Second, it is a triple alloy, not of steel with chromium alone, but of 85 steel with chromium and nickel. Third, it is, by virtue of a large chromium ingredient, a flame-resisting steel, and is therefore a material apart from those hard and tool-proof steels used as vault plates, in the 90 compounding of some of which the inclusion of small quantities of chromium has been proposed. Fourth, the chromium ingredient ranges from 10% upward, accompanied with a nickel ingredient of 2% and 95 upward. The upper limit to the amount of chromium is still the point at which the steel ceases to be workable, or (more correctly stated) the point at which the cost of production forbids going higher. An alloy 100 containing chromium 25%, with nickel 15%, showed under test flame-resisting quality three times better than cast iron; while other alloys having a chromium content ranging from 30% to 35% and a nickel 105 content of 12% to 15% were even better. These last named mixes are near the present practical maximum limit. I do not however mean to limit my invention to these figures, for with the development of mill operations 110 it may be possible presently to go higher.

The range of preferred composition under existing limitations upon mill operation is, chromium, 10 to 25%, nickel, 2 to 15%.

5 The carbon content of the steel should be low; other usual adulterants and metalloids present in small percentages in various steels, are in their presence or absence unrelated to the present invention. That is 10 to say, the invention may be practised upon steel of varying character and quality, so far as concerns these adulterants.

It further appears that the steel of my 15 invention is in marked degree resistant of attack by acid; it is then in the category of "stainless steel." This quality further adapts it to use not only for the heavy 20 protecting walls of safes, etc., but also for forming the lighter partitions and safe deposit boxes and drawers within; for the parts made of this material may be kept bright, even under difficult atmospheric conditions. And the bright and clear appearance of such structure is a not inconsiderable matter.

25 The particular way in which my improved vault plate is built into the safe structure, or the particular manner it may

be combined with other plates of tool-resisting or of other character, forms no part 30 of my present invention.

I claim as my invention:

1. A vault plate formed of a nickel-chromium-steel alloy, in which the chromium content is at least 10%, substantially as 35 described.

2. A vault plate formed of a nickel-chromium-steel alloy, in which the chromium content is at least 10% and the nickel content at least 2%, substantially as de- 40 scribed.

3. A vault plate formed of a nickel-chromium-steel alloy, in which chromium is between 10% and 25% and nickel between 2% and 15%, substantially as described. 45

4. A vault plate formed of a nickel-chromium-steel alloy, in which steel is the dominant component and the chromium content is at least 10%, substantially as de- 50 scribed.

In testimony whereof I have hereunto set my hand.

CHARLES MORRIS JOHNSON.

Witnesses:

BAYARD H. CHRISTY,  
FRANCIS J. TOMASSON.